

April 12, 1927.

1,624,338

C. R. HANNA

TELEPHONE RECEIVER

Filed Aug. 28, 1924

Fig. 1.



Fig. 2.



Fig. 3.



Fig. 5.



Fig. 4.



WITNESSES:

*A. L. Jeffrey*  
A. L. Jeffrey  
A. P. Fine Line

INVENTOR

Clinton R. Hanna

BY  
*Berkeley Barr*  
ATTORNEY

## UNITED STATES PATENT OFFICE.

CLINTON R. HANNA, OF WILKINSBURG, PENNSYLVANIA, ASSIGNOR TO WESTINGHOUSE ELECTRIC & MANUFACTURING COMPANY, A CORPORATION OF PENNSYLVANIA.

## TELEPHONE RECEIVER.

Application filed August 28, 1924. Serial No. 734,604.

My invention relates to telephone receiver devices and particularly to telephone receivers having permanent magnets.

One object of my invention is to produce a telephone receiver device in which full utilization is made of the properties of steels which have high coercive force.

In the steel, of which the permanent magnet in the telephone receiver disclosed herein is made, the changes in magnetic induction, corresponding to the small changes in impressed magneto-motive force, which are superposed upon the permanent magnetomotive force, are accompanied by greater losses than in steels heretofore used. Another object of this invention is to provide a structure in which said losses are largely avoided.

Another object of my invention is to produce a telephone receiver having a minimum amount of permanent-magnet steel therein.

Another object of my invention is to produce a telephone receiver having a path for the variable magnetic flux, distinct from the source of the permanent flux.

Another object of my invention is to produce a telephone receiver of minimum weight.

Another object of my invention is to produce a telephone receiver device capable of greater efficiency of translation of vibratory currents into sound than the devices of the prior art.

Telephone receivers ordinarily have a diaphragm mounted in a container case, within which are also placed a permanent magnet, pole pieces, attached thereto and adjacent the center of the diaphragm, electromagnet coils upon the pole pieces, and connecting and terminal blocks for the attachment of lead wires. It is customary for the permanent magnet to be made in a horse-shoe shape from such material as tool steel. With this construction there is a great deal of leakage flux and only a small portion of the total flux of the magnet passes through the pole pieces and the diaphragm. The present invention, by providing a short straight magnet, avoids this disadvantage.

In structures wherein the flux variations produced by the changing signal current are required to take place within the body of the permanent magnet, these flux variations are smaller than if they occurred in a magnetic circuit containing soft iron, only

This results in smaller vibrations of the diaphragm.

Also the large weight of the permanent magnets in the receivers as formerly built is objectionable, particularly when the telephone is one of a pair to be worn upon the head of an operator.

My invention provides means whereby a very short, small and light magnet is made to furnish sufficient magnetic flux for the operation of the telephone receiver. My invention further comprises means whereby the above-mentioned disadvantage of the permanent-magnet steel is avoided.

Other objects and structural details of my invention will be apparent from the following description, when read in connection with the accompanying drawing, wherein:

Fig. 1 is a perspective view of the permanent magnet and pole pieces in my invention,

Fig. 2 is a perspective view of an alternative construction.

Fig. 3 is a view partly in section of the magnetic circuit embodying my invention,

Fig. 4 is a view in sectional elevation of an embodiment of my invention, and

Fig. 5 is a diagram showing curves used in the explanation of the invention.

A permanent magnet 1 of a material such as cobalt steel which has a high coercive force, has attached to its pole the pole pieces 2 and 3. The pole pieces 2 and 3 are of L-shape and the lower portions of the L's are turned toward each other underneath the permanent magnet 1. The lower portions of the L's are separated from the permanent magnet 1 by a spacer 4, of non-magnetic material, preferably insulation. The pole pieces 2 and 3 do not quite meet below the spacer 4, but leave an air-gap 5 between their ends.

A diaphragm 6, shown in Figs. 3 and 4, is adjacent the upper ends of pole pieces 2 and 3.

Three paths for magnetic flux are provided. One path comprises the permanent magnet 1, the pole piece 2, the air-gap 5, and the pole piece 3, back to the permanent magnet 1.

A second path for magnetic flux comprises the permanent magnet 1, the upper portion of the pole piece 2, an air gap 7 between the pole piece and the diaphragm, the diaphragm 6, a second air-gap 8, the upper por-

tion of the pole piece 3 and permanent magnet 1. A third path for magnetic flux comprises the pole piece 2, the air gap 5, the pole piece 3, the air gap 8, the diaphragm 6, the air-gap 7, and the pole piece 2.

The receiver is mounted in a case 9, shown in Fig. 4. The diaphragm 6 is held in place by the cover 11, and the electromagnet coils 12 and 14 are positioned upon the pole pieces 2 and 3. The pole pieces 2 and 3 and the spacer 4 are held in place by the fastening means 15 and 16 and the binding posts 17 and 18 are provided for the attachment of the connector wires 19 and 20. The windings 12 and 14 may be wound on full sized ends of the pole pieces as in Fig. 1 or the pole pieces may have shoulders, as in Fig. 2, to position the windings.

In the operation of my device, the diaphragm 6 is attracted by the permanent magnet flux from the magnet 1 passing through the second of the above-described magnetic paths. Varying flux is induced in the third-mentioned magnetic circuit by the fluctuating currents in the coils 12 and 14. This flux produced by the fluctuating currents acts to increase or decrease the force acting upon the diaphragm 6, thereby causing it to move and to produce sounds.

Because the permanent magnet 1 is short, the leakage of the permanent magnetic flux is a minimum. The magnet 1 is made of a steel which has high coercive force.

In order to make clear how the selection of a steel of high coercive force results in the possibility of a short magnet, consider the change of the induction with alterations in the impressed magnetizing force. In the manufacture of the permanent magnet, it is made part of a closed magnetic circuit and a strong magnetomotive force applied. When the applied magnetomotive force is reduced to zero, the induction does not return to zero. Its value is the vertical intercept of the usual hysteresis loop represented by *oa* in Fig. 5.

When the magnet is removed from the closed magnetic circuit, the poles exert a de-magnetizing effect. This may be regarded as a negative magnetomotive force and so is represented in Fig. 5 by the abscissæ *H*, which are measured toward the left. The problem is to so choose the length and cross section of the permanent magnet that this de-magnetizing effect of the poles is of the most advantageous size.

The only magnetomotive force in the magnetic circuit, after the magnetizing process is over, is that of the poles. This must, therefore, not only reduce the induction within the permanent magnet from *oa* to its final value, say *bc*, but it must also cause the flux through the air gaps 5, 7 and 8 and the diaphragm. The magnitude of the flux through these air gaps being de-

cided upon, the required magnetomotive force is fixed.

Neglecting the effect of leakage through the sides of the permanent magnet we may write  $M=Hl$ , where  $M$  is the magnetomotive force in Gilberts,  $H$  is the de-magnetizing effect of the poles in Gilberts per centimeter and  $l$  is the length in centimeters.

If  $A$  be the area of cross section of the magnet and  $v$  its volume, we have

$$v = A l = A \frac{M}{H}$$

and, representing the induction by  $B$  and the flux by  $\Phi$ , we may multiply both terms of the fraction by  $B$  and obtain

$$v = \frac{MBA}{BH} = \frac{M\Phi}{BH}$$

The magnetomotive force  $M$  and the flux  $\Phi$  being fixed by the required conditions in the air gaps, this equation shows that the volume will be a minimum when  $BH$  is a maximum.

The curve II in Fig. 5 shows how the product  $BH$  changes with different values of  $B$ . It will be apparent, from inspection thereof, that the maximum value of the product occurs near the point *d*, for which  $B=6000$ .

Therefore, dividing the flux  $\Phi$  by 6000 gives the most desirable area of cross section. The length is then found by dividing the volume, determined by considerations stated above, by the cross section.

A numerical example is inserted to make the foregoing discussion concrete. In a receiver of the type illustrated in Fig. 4, the flux in the air gap 7 should be about 300 Maxwells. The reluctance of the magnetic circuit, through the permanent magnet and the diaphragm is ordinarily such that a magnetomotive force of 180 Gilberts is required to produce the 300 Maxwells of flux therein.

The flux  $\Phi$  in the magnet must supply not only these 300 Maxwells but also the flux through the shunt path including the air gap 5. This is some five times as great. The total flux in the permanent magnet is, therefore, 1800 Maxwells.

The product of the flux  $\Phi$  by the magnetomotive force  $M$  is, therefore,  $1800 \times 180 = 324,000$ . If this be divided by  $BH$  we shall obtain the volume. The induction  $B$  must be about 6000, because curve II shows a maximum at that ordinate. The value of  $H$  corresponding to  $B=6000$  is shown by curve I to be 153. The product  $BH$  is, therefore,  $6000 \times 153 = 918,000$ . Dividing 324,000 by 918,000 gives the volume of the magnet as 0.353 cubic centimeters.

The flux, 1800 Maxwells, when associated with an induction of 6000 Gausses, gives

1800  $\div$  6000 = 0.3 square centimeters for the area of cross section of the permanent magnet. The volume divided by the cross section gives the length,  $0.353 \div 0.3 = 1.177$ .  
 5 Again, the magnetomotive force, 180 Gilberts, being associated with 153 Gilberts per centimeter for the value of  $H$ , we have  $180 \div 153 = 1.176$  centimeters for the length of the magnet which agrees with the length as determined above.

10 The surprisingly small values for the volume and length of the magnet are a consequence of two considerations; first, a material is selected for which the product  $BH$  is greater than for other materials, and then a shape of magnet is selected which corresponds to the maximum value of the product  $BH$ . This will be evident from the curves in Fig. 5, where I and II represent the relation between the quantities  $BH$ ,  $H$ , and  $B$  for a steel containing some 38% of cobalt, while the curves I' and II' represent these relations for a steel containing 2% of chromium. By selecting the cobalt steel and that value of  $B$  corresponding to the point  $d$  on the curve II, the resulting volume and length of the magnet are most advantageous.

15 The values of  $H$  represented by  $oe$  for the chromium steel and by  $of$  for the cobalt steel are the "coercive forces" for these two materials. It will be noticed that the steel having the greater coercive force is the one which also has the greatest maximum value 20 for the product  $BH$ . If a choice were being made between two materials having nearly the same coercive force, it might be that the maximum value of the product  $BH$  occurred in the material with the smaller coercive force. If such circumstances should arise, the steel to be selected is the one for which the product  $BH$  is largest, but ordinarily this is the one with the greatest coercive force.

25 The dimensions indicated by the foregoing discussion are not strictly followed. There is some leakage through the sides of the permanent magnet and, to allow for this the volume must be slightly greater. Also the theoretical length is a little greater than the distance between pole pieces in a telephone receiver of standard size and the convenience of manufacture, resulting from following standardized dimensions, has caused 30 a trifle shorter length to be adopted, although a volume somewhat greater than the theoretical magnitude must then be used.

35 The above theoretical discussion describes the removal of the permanent magnet from the closed magnetic circuit in which it was magnetized. In practice, the magnet 1 is magnetized in a closed magnetic circuit of which the pole pieces 2 and 3 form a part and the permanent magnet is left in contact 40 with the pole pieces at all times, after the

original magnetization. If it were removed from them, the de-magnetizing effect of the poles would bring the induction down to some such point as  $g$  (Fig. 5). Then, upon placing the magnet between the pole pieces, 45 the induction would increase, not to the value  $e$  as desired, but to some value such as  $h$ , which is too small.

50 The magnetic circuit through air gaps 5, 7 and 8, in series, provides a path for the varying flux produced by the coils 12 and 14 which does not extend through the permanent magnet 1. Consequently, the small response of the material of the magnet 1 to the fluctuations in magnetomotive force, 55 does not cause any diminution of the changes which result from the changing current in the coils.

60 Although I have shown only one embodiment of my invention in the accompanying drawing, it is capable of various changes and modifications without departing from the spirit thereof and it is desired, therefore, that only such limitations shall be imposed thereon as are indicated in the prior art or 65 in the appended claims.

I claim as my invention:

1. A telephone receiver device, comprising a diaphragm and a magnetic circuit, including pole pieces, air gaps, said diaphragm and a permanent magnet, the length of said permanent magnet being no greater than the distance between portions of said pole pieces adjacent said diaphragm.

2. A telephone receiver device, comprising a diaphragm and a magnetic circuit, including pole pieces, air gaps, said diaphragm and a permanent magnet, the volume of said permanent magnet being sufficient to provide flux across the air gaps, of the magnitude needed to properly work the diaphragm, and the cross section of the permanent magnet being such that the magnetic induction therein has such a value that the said flux is obtained in a length no greater than that between the portions of said pole pieces adjacent said diaphragm.

3. A telephone receiver device comprising in combination a diaphragm, pole pieces co-operating therewith, positioned nearer the center of said diaphragm than one-half the radius thereof, coils co-operating with said pole pieces and supplied with fluctuating current, a permanent steel magnet of high-coercive-force and of a length substantially equal to the separation of said pole pieces adjacent the diaphragm, and a container case co-operating therewith.

4. A magnetic circuit for a telephone receiver, including a diaphragm, pole pieces cooperating with the diaphragm to form an approximately rectangular magnetic circuit, and a permanent magnet within the rectangle and constituting part of the magnetic circuit.

5. A magnetic circuit for a telephone receiver, including a diaphragm, pole pieces cooperating with the diaphragm to form an approximately rectangular magnetic circuit and a permanent magnet crossing the interior of the rectangle the shorter way, wholly within the rectangle, and constituting part of the magnetic circuit.
6. A magnetic system for a telephone receiver, comprising two L-shaped pole pieces with corresponding arms turned toward each

other, a coil on the other arm of each pole piece, a diaphragm adjacent to the ends of said last-named arms a permanent magnet parallel to said first named arms and a non-magnetic spacing block between said magnet and said first-named arms. <sup>15</sup>

In testimony whereof, I have hereunto subscribed my name this 22nd day of August, 1924.

CLINTON R. HANNA.